

# UNITED STATES PATENT OFFICE.

ALADAR PACZ, OF CLEVELAND HEIGHTS, OHIO.

## PROCESS FOR IMPROVING FERROUS METALS.

1,396,276.

Specification of Letters Patent.

Patented Nov. 8, 1921.

No Drawing.

Application filed April 16, 1920. Serial No. 374,261.

To all whom it may concern:

Be it known that I, ALADAR PACZ, a citizen of the United States, residing at Cleveland Heights, in the county of Cuyahoga and State of Ohio, have invented a certain new and useful Improvement in Processes for Improving Ferrous Metals, of which the following is a full, clear, and exact description.

10 This invention relates to the treatment of ferrous metals for the purpose of scavenging or deoxidizing the same, and also of producing certain properties and qualities therein, the better to fit them for certain 15 commercial purposes. In the manufacture of iron and steel it is customary to add to the molten metal certain substances, frequently called deoxidizers or scavengers, such as metallic manganese, titanium and 20 the like, which shall combine with any oxygen absorbed in or combined with the molten metal, themselves becoming oxidized and combining with the slag. Aluminum has been suggested for this purpose, but offers 25 the practical disadvantages of a too rapid reaction and of producing a product which is too infusible to separate and slag off readily and also too inactive chemically to 30 combine easily with other substances which might assist its fusion. I have also discovered that when by my improved process sufficient aluminum is added to molten iron to appear in the alloyed state in the 35 resulting product, a metallic composition is obtained which possesses very great resistance to oxidation at high temperatures as is frequently desirable in connection with furnace parts, heat treating boxes, carbonizing boxes, metallurgical tools, and the like 40 high temperature apparatus.

The essence of my invention or discovery is that if the aluminum be alloyed prior to its addition to the ferrous metal with a material quantity of silicon, both the above 45 described difficulties are avoided, the silicon serving to restrain the rapidity and violence of the reaction and also by its simultaneous oxidation to produce as a flux the comparatively fusible aluminum silicate instead of 50 the highly refractory aluminum oxide. Besides the character of the resulting metal is much improved whether all the aluminum be absorbed in process or whether enough be added so that some of the same persists 55 in the finished alloy.

In the performance of my said invention,

I preferably employ an alloy containing not less than about ten per cent. nor more than about forty per cent. of silicon, with the balance largely aluminum; although quantities of other metals such as manganese, 60 titanium, vanadium, tungsten, molybdenum, boron, iron, nickel, cobalt, or chromium can be employed if desired, or in case they occur as impurities as is sometimes the case. An 65 aluminum alloy containing the quantity of silicon above mentioned will react more slowly and will also produce a flux having a composition sufficiently near the theoretically correct relative amounts of silica and 70 alumina to fuse readily and separate easily. Besides such an alloy is normally sufficiently brittle to be readily disintegrated, thus facilitating its incorporation with the molten bath which may be effected either in the 75 customary direct manner or in the indirect manner described and claimed in my application filed March 18, 1920, Serial No. 366,968.

In case the added material is to be employed solely for the purpose of scavenging, only sufficient of the same is added as will be oxidized in process; while if a residue of the material be desired in the resulting metal for the sake of the peculiar properties 80 thereby conferred, a sufficiently greater quantity is added to effect this, after the necessary slag losses caused by the scavenging which always occurs. In the latter case I preferably produce an alloy containing between about one per cent. and about eighteen 85 per cent. of aluminum along with a corresponding amount of silicon depending upon the proportion of the same which accompanied the aluminum. The effect of the 90 aluminum is not only to enhance the resistance of the metal to high temperatures, but it also possesses certain valuable electrical and magnetic qualities such as that of lowering hysteresis losses in much the same manner 95 as silicon, and its use in company with silicon affords added advantages in this respect. It thus becomes valuable for the armatures of electromagnetic machines, for transformer cores, and in many kinds of 100 alternating current apparatus.

It will be understood that the essential feature of this invention is the employment in the relationship described, of an alloy containing silicon and aluminum, and that 110 this feature is not diminished by the addition of other materials thereto; also that

while I have pointed out a few important uses and purposes for which my discovery can be employed I am not limited to the same nor to any details except as specified in my claim.

Having thus described my invention, what I claim is:—

The method of producing an alloy of iron and aluminum which contains the steps of

first preparing an alloy of aluminum containing from about ten to about forty per cent of silicon, cooling and disintegrating the same and then adding it to a bath of molten iron.

In testimony whereof, I hereunto affix my signature.

ALADAR PACZ.